

Apr. 24, 1923.

1,452,954

W. A. BRAUN

PACK FOR ELECTRICAL HEATING ELEMENTS

Filed April 18, 1922

Fig. 1.



Fig. 2



William A. Braun, Inventor

By *A. G. Burns*

Attorney

## UNITED STATES PATENT OFFICE.

WILLIAM A. BRAUN, OF DOVER, OHIO, ASSIGNOR TO DOVER MANUFACTURING COMPANY, A CORPORATION OF OHIO.

## PACK FOR ELECTRICAL HEATING ELEMENTS.

Application filed April 18, 1922. Serial No. 555,257.

To all whom it may concern:

Be it known that I, WILLIAM A. BRAUN, a citizen of the United States of America, and resident of Dover, in the county of Tuscarawas and State of Ohio, have invented certain new and useful Improvements in Packs for Electrical Heating Elements, of which the following is a specification.

This invention relates to improvements in packs for electrical heating elements, especially for imbedding and insulating resistance wires within sad irons and other members to be heated.

In the prior art resistance wires have been used in packs placed in members to be heated through the action of electrical current passing through the resistance wires, such packs being formed of various materials and compositions of materials. It has been found that such materials and compositions have a tendency to deteriorate rapidly with use, and generally, are susceptible to a wide range of insulating efficiency, especially at different temperatures. Also, it has been difficult to provide packs of permanent dielectric properties that have also the desired capacity for conducting the heat of the resistance wire to the iron or member to be heated. A further difficulty ordinarily experienced is when a common pack is used the resistance wire tends to become oxidized to a detrimental extent which impairs the wire and reduces its efficiency, and it has been sought to overcome this difficulty by making use of highly refined and expensive metallic resistance members.

The objects of the present invention are: first, to produce a pack for an electrical heating member of low hygroscopic and high dielectric properties, and which also is highly efficient as a conductor of heat; second, to provide a pack for a resistance wire so constituted as to prevent the resistance wire becoming oxidized; and, third, to provide an efficient pack for resistance wires that may be constructed and applied by simple methods and without the usual application of heat at excessively high temperatures.

The above objects are accomplished by the use of the materials prepared and applied as hereinafter set forth, the accompanying drawings being illustrations of a sad iron in which a resistance member is shown im-

bedded in a pack embodying the present invention, and in which:

Figure 1 is a plan view of a sad iron partially broken away; and Fig. 2 is a longitudinal section, projected from Fig. 1.

The characters appearing in the description refer to parts shown in the drawings and designated thereon by corresponding characters:

The sad iron shown in the drawings is of usual construction and consists of a base 1 and a cover 2 that are secured together by a screw 3. The resistance member 4 is imbedded in the pack which is composed of a substratum 5 and superstratum 6 of cement, there being a cover 2 which affords the required added weight to the iron and serves also to reserve heat.

The invention comprises the pack composed of cement that is constituted of a mixture of refractory material, clay, and boracic acid, in relative proportions as per the following tabulation:

|                     | Per cent. |
|---------------------|-----------|
| Refractory material | 83        |
| Clay                | 12        |
| Boracic acid        | 5         |

The refractory material employed is such as "alundum fines" commonly known in the art, or may be such other hard granular or pulverulent material of similar character which is possessed of high thermal conductivity and high dielectric properties.

The clay herein used as an agent for holding the pulverulent refractory material suspended in the mixture, may be of any suitable character, such, for example, as Klingenberg clay which has been found satisfactory.

The boracic acid when introduced into the mixture is in the form of powder.

In preparing the cement, the ingredients are placed in a pebble mill with water approximately equal in quantity to half of the amount of powder, by weight, and therein is ground and worked into a plastic mass. The composition thus formed is then placed in a suitable mixing machine and agitated until used.

In making the pack, a substratum 5 is formed of the plastic cement in the hollow base of the iron, and while the substratum 5 is still in a plastic state the resistance wire

4 is partially imbedded therein and held in place until the substratum becomes dry and hard. The superstratum 6 of the plastic cement is then formed over the substratum 5 and resistance wire, completely covering the same. After the pack is thus formed, the cover 2 is clamped in place upon the pack, while plastic, with the terminals 7 of the resistance wire extending through corresponding openings 8.

An especial feature of the invention is that the boracic acid in the mixture becomes melted, forming boric oxide ( $B_2O_3$ ), when the temperature of the pack is raised by the 15 action of the electrical current passing through the resistance wire, which saturates the pack during the initial heating thereof so that the granular particles and the resistance wire become coated therewith and 20 the interstices between the particles and about the wire become filled. In this manner the pack is rendered exceedingly dense and its hygroscopic tendency is correspondingly reduced and its dielectric property conse- 25 quently is preserved. Also, the intimate coating thus formed upon the resistance wire prevents oxidation thereof so that its life is indefinitely protracted, and admits of the use of an ordinary and inexpensive resis- 30 tance wire.

It has been customary to initially subject 35 packs containing resistance members to very intense heat as well as great pressure for the purpose of increasing the dielectric efficiency of the pack. While such methods may 40 improve the insulation afforded the resistance member by the pack, the resistance member is impaired by the excessive heat in the operation. Also, packs that have been subjected to such excessive heat are more or less per-

vious and tend to absorb moisture from the atmosphere when not in use, which may occasion leakage or grounding when the resistance wire is again charged with electric current. In the present invention, however, 45 the initial heating of the pack is carried out at approximately the ordinary working temperature of the heating element without injury, and the pack is rendered practically imperious so that absorption of moisture 50 and consequent "grounding" is obviated. Also, in the present instance, the pack adheres to the resistance wire, and iron in which the pack is formed, without the usual application of great pressure, and the ordinary tendency of the pack to crumble and deteriorate is greatly reduced. 55

The materials forming the cement mixture and their relative proportions, set forth herein as an example for carrying out the 60 invention, are subject to such substitutions and variations of proportions as skill in the art affords, and therefore, my invention is extensive thereto.

What I claim is:—

1. A heating unit comprising a pack formed of a mixture of refractory material, clay and boracic acid, and an electrical resistance member encased in the pack.

2. In an electrically heated unit having a 70 resistance member, a pack encasing the member and being composed of pulverulent refractory material, clay and boracic acid.

In testimony whereof I affix my signature, in presence of two witnesses.

WILLIAM A. BRAUN.

Witnesses:

ZOE A. MUCKLEY,  
A. WENGER.